

## UNITED STATES PATENT OFFICE

WILHELM CHRIST, OF OFFENBACH-ON-THE-MAIN, GERMANY, ASSIGNOR TO GENERAL ANILINE WORKS, INC., OF NEW YORK, N. Y., A CORPORATION OF DELAWARE

## PRODUCTION OF ICE COLORS

No Drawing. Application filed November 19, 1925, Serial No. 70,186, and in Germany December 1, 1924.

The present invention relates to the production of the so-called "ice-colors."

The production of ice-colors by means of those azo components which possess a definite substantive character is generally carried out by padding a cotton mass with a solution of the proper azo component, dehydrating as far as possible by squeezing, pressing, suction, or centrifuging, and then, 10 without drying, developing, while still moist, by means of a diazo compound. Even when dehydrated as completely as possible, the fiber always mechanically retains a not inconsiderable amount of the padding liquor. 15 Particularly in packed material and warp-beams the spaces between the material hold considerable quantities of the padding liquor whose removal is desired in the production of unobjectionable colors, which is particularly 20 important in the use of azo components having only weak substantive properties.

This invention is based on an improvement in the production of ice-colors by means of azo components whose character allows the 25 development of the padded articles in moist condition, which consists in removing the padding solution held by the material after padding or dehydration, by treatment with a rinsing solution which contains an electrolyte as an essential component. By the expression "electrolyte" as used herein is to be understood not only a salt, but also a caustic 30 soda solution.

The rinsing liquid may consist of a more 35 or less weak padding solution to which caustic soda solution and a salt have been added, or in case the azo component used has a pronounced substantive character, of merely a solution of a salt, which in certain circumstances is partly replaced with some caustic 40 soda, or merely of a dilute caustic soda solution. By subsequent development there are produced colors much faster to rubbing which cannot be obtained without the removal 45 of the padding solution not fixed on the fiber, so that the dyer working with less care can obtain unobjectionable colors with certainty.

The described process finds advantageous 50 use, for example, in the production of ice

colors by means of the arylids or arylendi-imines of 2,3-hydroxynaphthoic acid (see U. S. Patent No. 1,099,108), or by the use of acetoacetyl or diacetoacetyl compounds of amino bases, as described in British Patents 55 Nos. 211,772 and 211,814, as well as in all cases in which there is used an azo component whose substantive character allows the development of the padded article in moist condition. 60

A further important advantage of the herein-described process lies in the fact that in this way, by the treatment with alkaline wash solutions, it is possible to remedy any possible injuries produced from the padding material on the fiber due to the action of the air during centrifuging, suction, or continued standing, which possibly leads to the formation of streaky or weak colors. Since further centrifuging or suction is unnecessary, and 65 as a result the air cannot further come into play, there is obtained in this way colors 70 wholly devoid of objection.

In using the described method of procedure, it is no longer necessary to add formaldehyde to the padding solution, for example, of 75 2,3 hydroxynaphthoic acid arylids, by means of which the padded articles are normally protected from the influence of the air, in so far as the process is carried out in the 80 hereinabove described manner following the dehydration step, and the color developed immediately thereafter. If, however, the mentioned solutions are used for washing before the centrifuging or suction operation, or if 85 it is necessary to allow the mass to stand for some time before the development of the color, it is best to work in such a way that padding is carried out with a padding solution containing no addition of formaldehyde, 90 and to add the formaldehyde to the mentioned displacing solution. In this way there is obtained in the simplest manner a padding bath free from formaldehyde, and which therefore possesses an unweakened permanency, while on the other hand the padded 95 yarns are rendered securely stable in the air.

The new process is useful in all processes 100 for the production of colors developed on the

fiber and marks an important technical development, since in this simple way unobjectionable and good colors fast to rubbing are obtained in all cases.

5

*Example 1*

30 kg. of yarn are padded in a bath with a solution containing 7 gr. of 2.3-hydroxynaphthoic acid anilid, caustic soda solution, and 7 c. c. of formaldehyde to the liter. The yarn is centrifuged and washed in the bath with a solution containing 0.5 gr. of 2.3-hydroxynaphthoic acid anilid, and further containing besides the amount of caustic soda necessary to keep it in solution 10 c. c. of caustic soda solution of 34° Bé. and 30 gr. of common salt per liter. After the washing, the washing solution is allowed to drain, and then the yarn is developed in the usual way.

20

*Example 2*

A warpbeam of 50 kg. is padded in an open or closed dyeing apparatus with a solution containing 2 gr. of 2.3-hydroxynaphthoic acid-beta-naphthalid and caustic soda per liter, pressed out with compressed air, and rinsed with a bath containing 40 gr. of common salt and 10 c. c. of caustic soda solution of 34° Bé. per liter. After rinsing it is again dehydrated by pressing and developed in the usual way.

30

*Example 3*

100 kg. of cross reels are padded in an apparatus according to the pack system, with a solution containing 1.5 gr. of bis-2.3-hydroxynaphthoyl-dianisidine and caustic soda per liter. After padding, the pack is rinsed with a liquor containing 12 c.c. of caustic soda solution of 34° Bé. per liter, and developed without centrifuging, in the ordinary manner.

40

*Example 4*

50 kg. of cotton yarn are padded in 1000 liters of a solution containing 2 gr. of 2.3-hydroxynaphthoylaminohydrochinondimethylether per liter and caustic soda. The padding bath is free from formaldehyde. After padding it is allowed to drain and the padded article is placed in a rinsing bath containing 50 gr. of common salt, 10 c. c. of caustic soda solution of 34° Bé. and 2 c. c. of formaldehyde per liter, removed after the rinsing centrifuged and developed in the usual way.

50

In the following claims the term "rinsing liquid" is intended to comprise only such aqueous liquids as contain the padding constituent, if at all, only in concentrations substantially less than the concentration of padding constituent in the liquid contained in the goods coming from the padding solution.

60

I claim:

65

1. In processes of producing ice colors on

textile materials from azo components, the character of which allows the development of the padded material in moist condition, the step comprising treating the padded material with a rinsing liquid containing a non-acidic electrolyte.

70

2. In processes of producing ice colors on textile materials from azo components, the character of which allows the development of the padded material in moist condition, the step comprising treating the padded material with a rinsing liquid containing a caustic alkali.

75

3. In processes of producing ice colors on textile materials from azo components, the character of which allows the development of the padded material in moist condition, the step comprising treating the padded material with a rinsing liquid containing a caustic alkali and an alkali metal salt.

80

4. In processes of producing ice colors on textile materials from azo components, the character of which allows the development of the padded material in moist condition, the step comprising treating the padded material with a rinsing liquid containing a caustic alkali, an alkali metal salt and formaldehyde.

85

5. In processes of producing ice colors on textile materials from azo components, the character of which allows the development of the padded material in moist condition, the step comprising treating the padded material with a rinsing liquid containing a non-acidic electrolyte and the padding solution in a concentration substantially less than that of the original padding liquor.

90

6. In processes of producing ice colors on textile materials the step comprising treating the textile material, padded with a 2-3-hydroxynaphthoic acid arylid compound, with a rinsing liquid containing a non-acidic electrolyte.

95

7. In processes of producing ice colors on textile materials the step comprising treating the textile material, padded with a 2-3-hydroxynaphthoic acid arylid compound, with a rinsing liquid containing a caustic alkali.

100

8. In processes of producing ice colors on textile materials the step comprising treating the textile material, padded with a 2-3-hydroxynaphthoic acid arylid compound, with a rinsing liquid containing a caustic alkali and an alkali metal salt.

105

9. In processes of producing ice colors on textile materials the step comprising treating the textile material, padded with a 2-3-hydroxynaphthoic acid arylid compound, with a rinsing liquid containing a caustic alkali, an alkali metal salt and formaldehyde.

110

10. In processes of producing ice colors on textile materials the step comprising treating the textile material, padded with a 2-3-

115

hydroxynaphthoic acid arylid compound,  
with a rinsing liquid containing a non-acidic  
electrolyte and the padding solution in a con-  
centration substantially less than that of the  
original padding liquor.

• In testimony whereof, I affix my signature.

DR. WILHELM CHRIST.